

922,655.

C. E. WOLLE.  
MANUFACTURE OF CAR WHEELS.  
APPLICATION FILED JAN. 12, 1909.

Patented May 25, 1909.



WITNESSES:

Jos. A. Wolle.

Percival A. Reed.

INVENTOR

Charles E. Wolle,  
BY

Jas. C. Hobusmith  
ATTORNEY.

# UNITED STATES PATENT OFFICE.

CHARLES E. WOLLÉ, OF BURNHAM, PENNSYLVANIA.

## MANUFACTURE OF CAR-WHEELS.

No. 922,655.

Specification of Letters Patent.

Patented May 25, 1909.

Application filed January 12, 1909. Serial No. 471,894.

*To all whom it may concern:*

Be it known that I, CHARLES E. WOLLÉ, a citizen of the United States, residing at Burnham, in the county of Mifflin and State of Pennsylvania, have invented certain new and useful Improvements in the Manufacture of Car-Wheels, of which the following is a specification.

My invention relates to the manufacture of car wheels and it has particular relation to the hardening of the tread and flange of rolled steel car wheels.

Heretofore, in view of the previous satisfactory performance of steel tired car wheels, the advent of the rolled steel was received with great satisfaction as it was believed that these wheels would embody all the good points of the steel tired wheel as well as having the additional features of integral construction, better hubs and webs, lower cost of production and other points which are well known to those skilled in the art. It has been found in practice, however, that in a number of instances the rolled steel wheel did not have the expected longevity or "mileage", due to the flange and tread being too soft, this fault being inherent and possibly resulting from the nature of the steel required to make a rolled wheel or from the process of manufacture not affording the proper or a sufficient manipulation of the rim of the wheel. To overcome this defect various attempts have been made to harden the rim of the wheel, it being well understood that it is desirable that the hub and web of the wheel be left soft. So far, however, none of the processes of hardening the rim of the wheel have been found to give satisfaction in practice. This invention therefore contemplates a method for hardening the wearing parts of rolled steel car wheels which it is believed will give the desired result.

The nature and characteristic features of my present invention will be more readily understood from the following description taken in connection with the accompanying drawing forming part thereof, which is a central sectional view of a rolled steel car wheel with a form of apparatus for carrying out my invention shown in connection therewith, the same being assembled in condition for immersion in a hardening bath.

Referring to the drawing, 1 is a rolled steel car wheel of the usual type. 2 and 3 are top and bottom convex cover plates which engage the wheel at the rim and incase the hub

and web of the wheel within a closed chamber. The lower cover plate 3 is provided with a series of feet 5 to enable it to rest in a stable horizontal position. Secured to the center of the lower cover plate 3 is an upwardly extending bolt 6 which passes through the bore of the wheel 1 as well as through an aperture 7 in the center of the upper cover plate 2. The entire structure is locked together to clamp the rim of the wheel between the edges of the cover plates 2 and 3 by means of a tapered key 8 which passes through a slot 9 in the bolt 6, the upper edge of the key 8 bearing against the upper end of slot 9 and the lower edge of key 8 bearing against a washer 10 interposed between it and the upper surface of the upper cover plate 2. The upper end of bolt 6 may be provided with an eye bolt 11 for engagement by suitable tackle for handling the assembled structure.

In carrying out the process of my invention, the wheel, heated to a proper hardening heat, is secured in place between the cover plates 2 and 3, as hereinbefore described. The entire assembled structure is now plunged, in a horizontal position, into a bath of suitable hardening compound, being then raised and lowered repeatedly until cold. The wheel is preferably arranged between the cover plates with the flange side of the wheel uppermost, so that when immersed the hardening solution may run up against the flange, and not be forced away from the same by the heat, to thereby insure the proper hardening of the fillet between the flange and tread of the wheel. The edges of the cover plates are made true on their faces to fit the rim of the wheel, but it is not essential that an absolutely tight joint be had at this point as any of the hardening bath which might tend to pass through such of a crevice as might exist would be immediately vaporized by the heat of the wheel and thereby be prevented from reaching the web or hub of the wheel to improperly harden the same.

By the foregoing process there is produced a rolled steel wheel having its tread and flange properly hardened to resist wear, whereas the hub and web are left in a softer state, so that there is no danger of fracture when the wheel is forced on the axle or when the wheel is in service carrying a heavy load, especially around curves.

Having thus described the nature and characteristic features of my invention, what

I claim as new and desire to secure by Letters Patent is:

1. The process of treating rolled steel car wheels which consists in heating the wheel to a proper hardening heat, then incasing the hub and web of the wheel in a protective housing, and then immersing the entire structure in a hardening bath.
2. The process of treating rolled steel car wheels which consists in heating the wheel to a proper hardening heat, then incasing the hub and web of the wheel in a protective housing which engages the rim of the wheel and leaves the tread and flange exposed, and then immersing the entire structure in a hardening bath.
3. The process of treating rolled steel car wheels which consists in heating the wheel to a proper hardening heat, then incasing the hub and web of the wheel in a housing which engages the rim of the wheel and leaves the tread and flange exposed and which forms an air chamber within which the hub and web of the wheel are protected from the action of

the hardening bath, and then immersing the entire structure in a hardening bath.

4. The process of treating rolled steel car wheels which consists in heating the wheel to a proper hardening heat, then incasing the hub and web of the wheel in a protective housing, and then immersing the entire structure in a hardening bath with the wheel in a horizontal position.

5. The process of treating rolled steel car wheels which consists in heating the wheel to a proper hardening heat, then incasing the hub and web of the wheel in a protective housing, and then immersing the entire structure in a hardening bath with the wheel in a horizontal position and with the flange side uppermost.

In testimony whereof I have hereunto signed my name in the presence of two witnesses.

CHAS. E. WOLLE.

Witnesses:

CATHARINE C. McCUALEY,  
EUGENE F. McCABE.